# EUROPEAN PATENT SPECIFICATION

(11) **EP 0 057 316 B1**
(45) Date of publication and mention of the grant of the patent: **03.04.1985**
(21) Application number: 81305667.8
(22) Date of filing: 02.12.1981
(51) Int. Cl.: C22C 38/22, C22C 38/26, C22C 38/28

(54) **Low interstitial, corrosion resistant, weldable ferritic stainless steel and process for the manufacture thereof**
Ferritischer, rostfreier, korrosionsbeständiger, schweissbarer Stahl mit geringem Gehalt an Zwischengittersubstanzen und Verfahren zu seiner Herstellung
Acier inoxydable ferritique, à basse teneur en éléments interstitiels, soudable et résistant à la corrosion, et procédé pour sa fabrication

(30) Priority: 16.01.1981 US 225566
(43) Date of publication of application: 11.08.1982
(73) Proprietor: ALLEGHENY LUDLUM STEEL CORPORATION, Pittsburgh Pennsylvania 15222 (US)
(72) Inventor: McCunn, Thomas Humes, Lower Burrell Pennsylvania 15068 (US); Deverell, Harry Edward, Natrona Heights Pennsylvania 15065 (US)
(74) Representative: Sheader, Brian N.

## Description

The present invention relates to a low interstitial, corrosion resistant, weldable ferritic stainless steel with improved toughness and to a process for the manufacture thereof. More specifically, the present invention is directed to a low interstitial/corrosion resistant, Weldable ferritic stainless steel with a small addition of either columbium or titanium to improve the toughness when the maximum achievable cooling rate is limited.

A ferritic stainless steel must have superior pitting and crevice corrosion resistance in order to be used in certain chemical environments as for example in power plants exposed to sea water, and pulp and paper process equipment. Stainless steel containing 29% chromium and 4% molybdenum are highly resistant to crevice corrosion. These steels require a low level of interstitials, for example a total carbon plus nitrogen content of less than 0.025% by weight, to have good post-welding ductility and intergranular corrosion resistance. ,

The applications mentioned above. often require heavy gauge supporting products such as plate, as well as light gauge welded tubing such as condenser tubing. This equipment is often assembled through a welding process. The shape and size of the assembled equipment usually prevents the use of a final heat treatment or, if capable of a final heat treatment, the shape and size often severely limit the ability of the assembled equipment to cool rapidly from the heat treating temperature. Moreover, the toughness of the alloy decreases as the thickness increases and as the cooling rate decreases. This is illustrated in Figure 12 in a paper by H. E. Deverall entitled "Toughness Properties of Vacuum Induction Melted High-Chromium Ferritic Stainless Steels", published in ASTM STP 706, Toughness of Ferritic Stainless Steels, R. A. Lula_{;} Ed., American Society for Testing and Materials, 1980. The decrease in toughness decreases weldability such that the plate, which in some instances may be incapable of being water-quenched because of its size, might exhibit cracking during welding. Or, if the plate is water-quenched, the cooling rate because of the thickness of the plate may not be rapid enough to achieve suitable toughness such that the plate may exhibit cracking during welding. Therefore, better toughness must be achieved by some other means where water-quenching is impractical or where water-quenching does not achieve suitable toughness to improve the weldability of the various components comprising the final assembled structure.

Even if the final product is to be of light gauge, the conventional production methods require the cooling of thicker slabs and bands during processing. The cooling rates of these heavier section sizes is slow. Water-quenching would speed up the cooling process, however water-quenching is often impossible or impractical due to shape and size.

As the thickness of the product section increases, the toughness as measured by Charpy impact transition temperature decreases. Toughness is the ability of a metal to absorb energy by deforming plastically before fracturing. The transition temperature is the temperature at which the fracture which occurs from the impact is 50 percent shear (ductile) and 50 percent cleavage (brittle).

The toughness of the 29% chromium - 4% molybdenum alloy is low compared to substantially lower chromium alloys of an equivalent carbon and nitrogen content because of the high alloy content. The toughness of the 29% chromium - 4% molybdenum alloy is improved by water-quenching to speed up the cooling process instead of the slower air-cooling. However, in many cases the water-quenching process is not possible or practical to use, so a method is needed to improve the toughness of the steel in those situations where the maximum cooling rate is limited.

A 29% chromium - 4 %molybdenum ferritic stainless steel with a maximum carbon plus nitrogen content of 0.025% is disclosed in United States Patent No. 3,929,473. United States Patent No. 3,932,174 is a modification to which small amounts of other elements are added to achieve the same range of corrosion properties as United States Patent No. 3,929,473. However these patents do not teach the use of columbium or titanium.

United States Patent No. 3,807,991 teaches the addition of between 13 and 29 times the amount of nitrogen or between 0.065% and 0.363% columbium to a steel of 1 % molybdenum for improved toughness and intergranular corrosion resistance in the air-cooled condition. United States Patent 3,957,544 discusses the addition of titanium and columbium according to the equation %Ti,s+%CB,e=(%C+%N). The molybdenum content of the steels in these patents is lower than that of the present invention.

The presence of titanium and columbium in the steel reduces the susceptibility of a steel to intergranular attack, but the weldability of the steel is poor unless the level of interstitials is low. Molybdenum improves pitting and crevice corrosion resistance, but according to United States Patent 4,119,765 if molybdenum is present in an amount of over 3.5% and is combined with chromium, titanium, silicon or columbium, the notch toughness is reduced, especially in the as-welded condition. United States Patent 4,119,765 adds from 2%-4.75% nickel to improve the weldability of the steel. The amount of nickel must be regulated carefully so as to improve notch toughness and acid corrosion resistance without interfering with other properties.

A final reference is a paper entitled "Ferritic Stainless Steel Corrosion Resistance and Economy", by Remus A. Lula. The paper appeared on pages 24-29 of the July 1976 issue of Metal progress. This reference does not disclose the ferritic stainless steel of the present invention.

For the reasons noted hereinabove, the present invention is distinguishable from the references referred to.

An object of the present invention is to provide a low interstitial, corrosion resistant, weldable ferritic stainless steel with a high molybdenum content which exhibits improves toughness in heavier section thickness when the maximum achievable cooling rate is limited.

A further object of the present invention is to provide a low interstitial, corrosion resistant, weldable ferritic stainless steel with a high molybdenum content which exhibits improved toughness due to a small addition of either columbium or titanium.

In particular, this invention provides a low interstitial ferritic stainless steel which is corrosion resistant and weldable at room temperature. The improvement of the present invention being an addition of a small critical amount of columbium and/or titanium to improve the toughness of the steel in situations where water quenching is impossible or impractical.

The present invention provides a low interstitial, corrosion resistant, weldable ferritic stainless steel with improved toughness characterized in that it consists of, by weight percent: 25.0%-35.G% chromium, 3.6%-5.6% molybdenum, less than 3% nickel, less than 2% manganese, less than 2.0% silicon, less than 0.5% aluminum, less than 0.50% copper, less than 0.050% phosphorus, less than 0.05% sulfur, less than 0.01 % carbon, less than 0.02% nitrogen, the sum of the carbon and nitrogen being less than 0.025%, 0.05-0.50% of columbium and/or titanium, and the balance of iron.

The present invention further provides a process for the manufacture of ferritic stainless steel of improved toughness wherein said steel is hot rolled, annealed and cold-rolled to strip thickness, characterized in that the process comprises air-cooling from the annealing temperature before cold rolling a ferritic stainless steel consisting essentially of, by weight per cent: 25.0%-35.0% chromium, 3.6%-5.6% molybdenum, less than 3.0% nickel, less than 2.0% manganese, less than 2.0% silicon, less than 0.5% aluminum, less than 0.5% copper, less than 0.5% phosphorus, less than 0.05% sulfur, less than 0.01% carbon, less than 0.02% nitrogen, the sum of the carbon and nitrogen being less than 0.025%, 0.05%-0.50% of columbium and/or titanium, and the balance iron, so as to produce a steel with a Charpy impact transition temperature of below -17.8°C (0°F) as cold-rolled to a thickness of 1.575 mm (0.062 inches).

Chromium and molybdenum are preferably present in respective amounts of 28.5% to -30.5% and 3.75% to 4.75%. Columbium and/or titanium is present preferably in the amount of 0.05% to 0.20%. Manganese and silicon are each usually present in amounts of less than 1%. Aluminum, copper, phosphorous, and sulfur are present usually in amounts of less than 0.1 %. Carbon and nitrogen are present preferably in amounts of less than 0.008% and 0.016% respectively.

The advantages of the steel of this invention will be apparent from the following description which is illustrative of several aspects of the invention. This invention relates to a low interstitial ferritic stainless steel having a chromium content of between 25.0% and 35.0% and a molybdenum content of between 3.6% and 5.6%. A small amount of columbium or titanium of between 0.05% and 0.20% is added to the steel composition to improve its toughness when the maximum achievable cooling rate is limited.

Ingots from four heats were vacuum-induction melted to the compositions given in Table I.

The ingots were conditioned, heated to a temperature of 1121°C (2050°F) and hot rolled to a strip about 3.556 mm (0.140 in.) thick. The hot rolled band was annealed at a temperature of 1010°C (1850°F), and water-quenched and cold rolled to a thickness of 1.575 mm (0.062 in.). The strip was then annealed at a temperature of 1010°C (1850°F), water-quenched and TIG welded.

Four sets of transverse Charpy V-notch impact subsize specimens were taken, two from the hot rolled band and the others from the 1.575 mm (0.062 in.) thick strips. After annealing the specimens at a temperature of 1010°C (1850°F), the specimens were either water-quenched or air-cooled. The cooled specimens were then tested for toughness characteristics. The results of the tests are shown in Table II.

The transition temperature decreases with increasing columbium content in the air-cooled condition thus indicating that columbium acts against the detrimental effects on toughness of slow cooling. Although the impact transition temperatures of the air-cooled specimens are higher than those of the water-quenched specimens it can be seen from Table II that the difference in impact transition temperatures of an air-cooled and a water-quenched 1.575 mm (0.062 in.) thick steel strip is less than 55°C (100°F). Whereas the difference in impact transition temperature for prior art compositions is 133°C (240°F). However, in situations where water-quenching is impractical or in situations where the cooling rates achieved by water-quenching of heavy thickness sections approach or are slower than those of air cooling lighter thickness sections, the addition of columbium improves the toughness. The impact transition temperature of the 1.575 mm (0.062 in.) steel strip of a composition according to the present invention is below -17.8°C (0°F) whereas that of prior art composition A is 54°C (130°F). It is essential that the impact transition temperature of such a steel strip be below room temperature so that the steel strip will not crack upon welding. Steels of prior art compositions had to be water-quenched before cold rolling in order to achieve the necessary toughness characteristics. The composition of this invention enables us to achieve good toughness characteristics by air-cooling the steel before cold-rolling instead.

Corrosion tests were also performed on the 1.575 mm (0.062 in.) thick strip in the as welded condition and on the base metal specimens which were heat treated at 1232°C (2250°F) and air-cooled to simulate the heat affected zone upon welding a heavier thickness. The specimens 25.4 mmx50.8 mm (1 in.x2 in.) were exposed to a boiling solution of ferritic sulfate-50% sulfuric acid for 120 hours according to ASTM A262 Practice B for intergranular corrosion testing. The corrosion rates are given in Table Ill.

The results of additional tests of the mechanical properties of the steel in the welded condition are shown in Table IV.

## Claims

1. A low interstitial, corrosion resistant, weldable ferritic stainless steel with improved toughness characterized in that it consists of, by weight percent: 25.0%-35.0% chromium, 3.6%-5.6% molybdenum, less than 3.0% nickel, less than 2.0% manganese, less than 2.0% silicon, less than 0.5% aluminum, less than 0.50% copper, less than 0.050% phosphorous, less than 0.05% sulfur, less than 0.01 % carbon, less than 0.02% nitrogen, the sum of the carbon and nitrogen being less than 0.025%, 0.05%-0.50% of columbium and/or titanium, and the balance of iron.

2. A low interstitial, corrosion resistant, weldable ferritic stainless steel with improved toughness according to claim 1 with a chromium content of from 28.5% to 30.5%.

3. A low interstitial, corrosion resistant, weldable ferritic stainless steel with improved toughness according to claim 1 or 2, with a molybdenum content of from 3.75% to 4.75%.

4. A low interstitial, corrosion resistant, weldable ferritic stainless steel with improved toughness according to claim 1, 2 or 3, with 0.05%-0.20% of columbium and/or titanium.

5. A low, interstitial, corrosion resistant, weldable ferritic stainless steel with improved toughness according to any one of the preceding claims with 0.05%-0.20% columbium.

6. A process for the manufacture of ferritic stainless steel of improved toughness wherein said steel is hot rolled, annealed and cold-rolled to strip thickness, characterized in that the process comprises air-cooling from the annealing temperature before cold rolling a ferritic stainless steel consisting essentially of, by weight per cent: 25.0%-35.0% chromium, 3.6%-5.6% molybdenum, less than 3.0% nickel, less than 2.0% manganese, less than 2.0% silicon, less than 0.5% aluminum, less than 0.5% copper, less than 0.5% phosphorous, less than 0.05% sulfur, less than 0.01 % carbon, less than 0.02% nitrogen, the sum of the carbon and nitrogen being less than 0.025%, 0.05%-0.50% of columbium and/or titanium, and the balance iron, so as to produce a steel with a Charpy impact transition temperature of below -17.8°C (0°F) as cold-rolled to a thickness of 1.575 mm (0.062 inches).

7. A process comprising welding a low interstitial, corrosion resistant, weldable ferritic stainless steel with improved toughness made according to the process of claim 6.

## Revendications

1. Acier inoxydable ferritique soudable, résistant à la corrosion, à faible teneur en éléments interstitiels et ayant une ténacité accrue, caractérisé en ce qu'il est formé, en pourcentages pondéraux, de 25,0 à 35,0% de chrome, de 3,6 à 5,6% de molybdène, de moins de 3,0% de nickel, de moins de 2,0% de manganèse, de moins de 2,0% de silicium, de moins de 0,5% d'aluminium, de moins de 0,50% de cuivre, de moins de 0,050% de phosphore, de moins de 0,05% de soufre, de moins de 0,01 % de carbone, de moins de 0,02% d'azote, la somme de l'azote et du carbone étant inférieure à 0,025%, de 0,05 à 0,50% de niobium et/ou de titane, et de fer pour le reste.

2. Acier inoxydable ferritique soudable, résistant à la corrosion, à faible teneur en éléments interstitiels et ayant une ténacité accrue selon la revendication 1, ayant une teneur en chrome comprise entre 28,5 et 30,5%.

3. Acier inoxydable ferritique soudable, résistant à la corrosion, à faible teneur en éléments interstitiels et ayant une ténacité accrue selon l'une des revendications 1 et 2, avec un teneur en molybdène comprise entre 3,75 et 4,75%.

4. Acier inoxydable ferritique soudable, résistant à la corrosion, à faible teneur en éléments interstitiels et ayant une ténacité accrue selon l'une quelconque des revendications 1 à 3, ayant 0,05 à 0,20% de niobium et/ou de titane.

5. Acier inoxydable ferritique soudable, résistant à la corrosion, à faible teneur en éléments interstitiels et ayant une ténacité accrue selon l'une quelconque des revendications précédentes, avec 0,05 à 0,20% de niobium.

6. Procédé de fabrication d'un acier inoxydable ferritique ayant une ténacité accrue, selon lequel t'acier est laminé à chaud, recuit et laminé à froid à l'épaisseur d'un feuillard, caractérisé en ce que le procédé comprend le refroidissement à l'air à partir de la température de recuit et avant laminage à froid, d'un acier inoxydable ferritique formé essentiellement, en pourcentages pondéraux, de 25,0 à 35,0% de chrome, de 3,6 à 5,6% de molybdène, de moins de 3,0% de nickel, de moins de 2,0% de manganèse, de moins de 2,0% de silicium, de moins de 0,5% d'aluminium, de moins de 0,5% de cuivre, de moins de 0,5% de phosphore, de moins de 0,05% de soufre, de moins de 0,01% de carbone, de moins de 0,02% d'azote, la somme du carbone et de l'azote étant infériure à 0,025%, de 0,05 à 0,50% de niobium et/ou de titane, et de fer pour le reste, afin que l'acier produit ait une température de transition au choc Charpy inférieure à -17,8°C, sous forme laminée à froid à une épaisseur de 1,575 mm.

7. Procédé comprenant le soudage d'un acier inoxydable ferritique soudable, résistant à la corrosion, à faible teneur en éléments interstitiels et ayant une ténacité accrue, fabriqué selon le procédé de la revendication 6.

## Patentansprüche

1. Korrosionsbeständiger, schweißbarer ferritischer, rostfreier Stahl mit geringem Gehalt an Zwischengittersubstanzen und gesteigerter Zähigkeit, dadurch gekennzeichnet, daß er besteht aus (Gew.-%): 25,0 bis 35,0% Chrom, 3,6 bis 5,6% Molybdän, weniger als 3,0% Nickel, weniger als 2,0% Mangan, weniger als 2,0% Silicium, weniger als 0,5% Aluminium, weniger als 0,5% Kupfer, weniger als 0,05% Phosphor, weniger als 0,05% Schwefel, weniger als 0,01% Kohlenstoff, weniger als 0,02% Stickstoff wobei die Summe aus dem Kohlenstoffgehalt und dem Stickstoffgehalt weniger als 0,025% beträgt, 0,05 bis 0,5% Niob und/oder Titan, Rest Eisen.

2. Korrosionsbeständiger, schweißbarer ferritischer, nichtrostender Stahl mit geringem Gehalt an Zwischengittersubstanzen und gesteigerter Zähigkeit nach Anspruch 1, mit einem Chromgehalt von 28,5 bis 30,5%.

3. Korrosionsbeständiger, schweißbarer ferritischer, rostfreier Stahl mit geringem Gehalt an Zwischengittersubstanzen und mit gesteigerter Zähigkeit nach Anspruch 1 oder 2 mit einem Molybdängehalt von 3,75 bis 4,75%.

4. Korrosionsbeständiger, schweißbarer, ferritischer, rostfreier Stahl mit geringem Gehalt an Zwischengittersubstanzen und gesteigerter Zähigkeit nach Anspruch 1, 2 oder 3 mit 0,05 bis 0,2% Niob und/oder Titan.

5. Korrosionsbeständiger, schweißbarer, ferritischer nichtrostender Stahl mit geringem Gehalt an Zwischengittersubstanzen mit gesteigerter Zähigkeit nach irgendeinem der vorhergehenden Ansprüche mit 0,05% bis 0,2% Niob.

6. Verfahren zum Herstellen des ferritischen, nichtrostenden Stahls mit verbesserter Zähigkeit, wobei der Stahl warmgewalzt, geglüht und auf Bandabmessung kaltgewalzt wird, dadurch gekennzeichnet, daß das Verfahren umfaßt ein Abkühlen an Luft von der Glühtemperatur vor dem Kaltwalzen eines ferritischen, rostfreien Stahls bestehend im wesentlichen aus (Gew.-%): 25,0 bis 35,0% Chrom, 3,6 bis 5,6% Molybdän, weniger als 3,0% Nickel, weniger als 2,0% Mangan, weniger als 2,0% Silicium, weniger als 0,5% Aluminium, weniger als 0,5% Kupfer, weniger als 0,05% Phosphor, weniger als 0,05% Schwefel, weniger als 0,01 % Kohlenstoff, weniger als 0,02% Stickstoff wobei die Summe aus dem Kohlenstoffgehalt und dem Stickstoffgehalt weniger als 0,025% beträgt, 0,05 bis 0,5% Niob und/oder Titan, Rest Eisen, so daß ein Stahl mit einer Charpy-Schlag-Übergangstemperaturvon weniger als 17,8°C (Grad F) im auf eine Dicke von 1,575 mm (0,052 Zoll) kaltgewalzten Zustand erhalten wird.

7. Verfahren umfassend das Schweißen eines korrosionsbeständigen, schweißbaren, ferritischen, nichtrostenden Stahls mit geringem Gehalt an Zwischengittersubstanzen und gesteigerter Zähigkeit, hergestellt gemäß des Verfahrens nach Anspruch 6.
